

Dec. 15, 1936.

W. SCHMIDT ET AL

2,064,323

PROCESS OF FORGING MAGNESIUM AND HIGH PERCENTAGE MAGNESIUM ALLOYS

Filed July 29, 1931

*Fig. 1.*



*Fig. 2a.*



*Fig. 2b.*



*Fig. 3.*



Walter Schmidt  
Hubert Altwicker  
INVENTORS

BY  
Hauffel Warland  
ATTORNEYS

## UNITED STATES PATENT OFFICE

2,064,323

## PROCESS OF FORGING MAGNESIUM AND HIGH PERCENTAGE MAGNESIUM ALLOYS

Walter Schmidt and Hubert Altwicker, Bitterfeld, Germany, assignors, by mesne assignments, to Magnesium Development Corporation, a corporation of Delaware

Application July 29, 1931, Serial No. 553,822  
In Germany August 16, 1930

## 8 Claims. (Cl. 78—12)

The present invention relates to a process of forging magnesium and high percentage magnesium alloys.

In the production of forgings, the material is so deformed as to obtain, concurrently with the shaping, a reduction of the individual grain size—an end which is desirable in view of the coincident improvement of mechanical properties.

Because of the hexagonal structure of magnesium it frequently occurs that forgings obtained by working magnesium and magnesium alloys are extensively oriented crystallographically. Such forgings thus necessarily vary in their capacity for resisting stresses, of differing direction, particularly as regards the ratio between the yield point of the forging under elongation and compression respectively. This is probably attributable to the peculiar conditions of deformation (translation, or twinning) of the individual hexagonal crystals of the metal. A capacity for resisting high stresses in only one direction is undesirable in a forging, since, ordinarily, the finished forging is subjected to stress components of differing direction. This leads to the problem of producing forgings of magnesium, and magnesium alloys, whose capacity for resisting tension and compression stresses, as far as practicable, is the same in all directions.

The present invention relates to a process for the production of magnesium forgings which have, as closely as possible, the same resistance to tension and compression stresses in every direction. According to the present invention the orientation of the mechanical properties in magnesium forgings is suppressed to a substantial extent by forging in such a manner that, during the deformation of the original ingot, the final shape and dimensions of the forgings are approached by stages, and by interposing, between those individual stages which serve to lead to the desired final shape, stages in which the forging is effected by blows in a direction at right angles to the direction of the blows effecting the main direction of deformation in view of the final shape. Of course, the main direction of deformation must always remain predominant; but the interposed changes of forging direction at right angles to the main direction prevent excessive crystallographic orientation, check slip of the crystals and/or retard twinning. In this way, a gradual approximation of the final shape is obtained. When, as is possible, the final shaping step is effected by swaging or die-pressing, it is advisable to select the lowest temperature possible (having in mind the shape of the die) so as

to prevent recrystallization of the irregular crystalline structure produced by the previous operations.

As a further advantage of the present invention, the forging process itself is facilitated. Since, in the case of magnesium and its alloys, the deformation substantially occurs by translation of the basal plane, continued deformation in one and the same direction would in combination with the uniform orientation of the crystals taking place under such deformation, lead, in a relatively short time, to a condition in which the arrangement of the individual crystals would hinder any further deformation in the same direction. This unfavourable effect is counteracted, in the present invention, by the opposing stages of directional deformation so that the finishing of the forging is facilitated. It is particularly advisable, in cases where the final shaping step is performed in a die, to select, as the last deformation stage prior to swaging or die-pressing, a stage in which the direction of deformation is opposed to the desired main direction of deformation in the die. If, for example, it is desired to form, in the die, an annular body, the dimensions of which are greater radially than axially, it is advisable to so forge the work piece that elongation in the radial direction takes place during die-pressing (the final stage of deformation). By this means the flow of the metal in the radial direction, when in the die, is substantially facilitated.

In order to clearly describe the nature of the present invention, reference is made to the accompanying drawing, which illustrates diagrammatically and by way of example a typical embodiment of the process of the present invention.

Referring to the drawing Fig. 1 is a view in elevation of a blank under deformation and represents the first stage of the process; Figures 2a and 2b, respectively, illustrate a lateral and an axial view of the piece, obtained from that shown in Figure 1, in the second stage of the process.

In Figs. 1, 2a and 2b, the broken lines indicate the shape of the block when the particular stage in question is started, whereas the full lines represent the final shape of the block on termination of such stage; and Figure 3 represents a side view of the final shape of the object.

Referring to Fig. 1, a is the original blank, which is first forged, by an upsetting operation (see arrow / indicating the direction of deformation), into a body shaped as at b. As will be seen from the drawing, this upsetting operation serves to compress the original blank or billet so as to produce radial outward flow of the

metal in all directions substantially normal to the direction of the applied force  $f$ . This body  $b$  is then turned through  $90^\circ$  and, while being continuously rotated on its axis (see Fig. 2b and 5 note the arrow  $f'$  indicating the direction of rotation), is deformed in a direction which is transverse to the original direction of deformation by repeated blows in a direction shown by arrow  $f$  thus effecting an elongation of the upset block. 10 Due to the continuous rotation of the body  $b$  on its axis, the blows applied in the direction indicated by arrow  $f$  are effective to apply radial pressure at a plurality of points of the previously deformed billet (body  $b$ ), and it will be noted 15 that such radial pressure is applied in a direction which is always substantially parallel to the directions of metal flow in the initial compressing operation shown in Fig. 1. By several repetitions of these operations, namely alternate 20 upsetting and elongation, the upsetting being always slightly predominant, a body of the form shown in Fig. 3 is finally obtained, the mechanical properties of which are substantially the same in the direction  $x$ ,  $y$  and  $z$ . The final 25 shape is then imparted to this body by forging in the die.

Several examples of the application of the process of the present invention will now be given.

30

*Example 1*

For producing a forged crank case for a radial engine, a known magnesium alloy containing about 8 percent of aluminium may be employed. In such a piece it is necessary that the capacity for resisting stress, both as regards tension and compression, should be as closely as possible the same in all directions. A crude ingot, 300 mms. in diameter and 600 mms. high, 35 is cast from this alloy and is then upset, as an upright cylinder, at 280-400° C., in the forging press, until the height has been reduced by 30 percent. The ingot is then turned on its axis, through  $90^\circ$  from the original direction, and the 40 deformation is continued, by forging transversely to the first direction of deformation, the ingot being continuously rotated on its original axis, until the diminution produced in the original height of the cylinder in both operations is reduced to about 15 percent. The ingot is then again turned through  $90^\circ$ , and the forging is continued in the same way, by alternate upsetting and elongation, though, in view of the final shaping, the upsetting predominates in each case. 45 After the original height of the cylinder has been reduced by about 70 per cent in this manner, the final shaping is effected in the die at 280° C. The result attained by this process is that the finished piece exhibits practically the same elongation yield point both in the direction of the original cylinder axis and at right angles thereto, namely about 16-18 kgs. per square millimeter. At the same time the compression yield point is very near the tensile yield point, having been ascertained to be 14-16 kgs. per square 50 millimeter in both directions.

*Example 2*

The same magnesium alloy as referred to in 70 Example 1 is employed for making a forged aircraft propeller. It is necessary that a work piece of this kind should also, as far as possible, have the same resistance to tension and compression in every direction. Consequently, it is particularly desirable that the blade possesses good 75

mechanical properties at right angles to its axis, because the transverse or oscillatory stresses occurring at the hub act in that direction. Hence, the highly stressed portion in the vicinity of the hub is formed in stages, by alternate forging in 5 directions differing by right angles, with gradual approximation to the final shape, in the manner described in Example 1. In the case of the blade, too, the forging is performed by alternate elongation, upsetting and broadening. The final 10 shaping, particularly as regards the pitch of the propeller blade, is effected, in a known manner, by pressure in the die.

We claim:

1. A process of forging magnesium and high 15 percentage magnesium alloys which comprises the steps of compressing a billet so as to produce radial outward flow of the metal in all directions substantially normal to the direction of the applied force, and applying radial pressure 20 at a plurality of points of the deformed billet and substantially parallel to the directions of metal flow in the initial compressing operation so as to compensate for the major part of the deformation produced in the first step. 25

2. A process of forging magnesium and high percentage magnesium alloys which comprises the steps of compressing a billet so as to produce flow of the metal in a direction to produce the shape desired, and applying pressure to the 30 deformed billet substantially parallel to the direction of metal flow in the initial compressing operation so as to compensate for the major part of the deformation produced in the first step. 35

3. As a new article of manufacture, a forged blank of metal, in which magnesium largely predominates, having the substantially unoriented crystal grain structure throughout characterizing magnesium which has been compressed to 40 flow the metal radially outward and thereafter subjected to pressure substantially parallel to the directions of metal flow in the initial compressing operation, said blank by virtue of the unoriented crystal structure being further 45 characterized by a resistance to mechanical stresses substantially equal in all directions.

4. As a new article of manufacture, a forged blank of metal, in which magnesium largely predominates and containing about 8 per cent of 50 aluminum, said blank having the substantially unoriented crystal grain structure throughout characterizing magnesium which has been compressed to flow the metal radially outward and thereafter subjected to pressure substantially 55 parallel to the directions of metal flow in the initial compressing operation, said blank by virtue of the unoriented crystal structure being further characterized by a resistance to mechanical stresses substantially equal in all directions. 60

5. A process of forging magnesium and high percentage magnesium alloys in stages which comprises subjecting a billet to forging stages in which the billet is compressed so as to produce flow of the metal at substantially right angles 65 to the compressive forces, and in a direction to produce the shape desired, and interposing between said forging stages intermediate forging stages in which pressure is applied to the deformed billet substantially parallel to the direction of metal flow in the first-named forging stages, the deformation produced by said intermediate forging stages compensating for the major part of the deformation produced in the 70 said first-named forging stages. 75

6. A process of forging magnesium and high percentage magnesium alloys in stages which comprises subjecting a billet to forging stages in which the billet is compressed so as to produce flow of the metal at substantially right angles to the compressive forces, and in a direction to produce the shape desired, and interposing between said forging stages intermediate forging stages in which pressure is applied to the deformed 5 billet substantially parallel to the direction of metal flow in the first-named forging stages, the deformation produced by said intermediate forging stages compensating for the major part of the deformation produced in the said first-named forging stages, the final stage of deformation being effected at the lowest temperature compatible with plastic deformation.
7. A process of forging magnesium and high percentage magnesium alloys in stages which comprises subjecting a billet to forging stages in which the billet is compressed so as to produce flow of the metal at substantially right angles to the compressive forces, and in a direction to produce the shape desired, and interposing between said forging stages intermediate forging stages in which pressure is applied to the deformed billet substantially parallel to the di- 10 15 20 25

rection of metal flow in the first-named forging stages, the deformation produced by said intermediate forging stages compensating for the major part of the deformation produced in the said first-named forging stages, the final stage 5 of deformation being effected by swaging.

8. A process of forging magnesium and high percentage magnesium alloys in stages which comprises subjecting a billet to forging stages in which the billet is compressed so as to produce flow of the metal at substantially right angles to the compressive forces, and in a direction to produce the shape desired, and interposing between said forging stages intermediate forging stages in which pressure is applied to the deformed billet substantially parallel to the direction of metal flow in the first-named forging stages, the deformation produced by said intermediate forging stages compensating for the major part of the deformation produced in the said first-named forging stages, the final stage 10 15 20 25 of deformation being effected by swaging at the lowest temperature compatible with plastic deformation.

WALTER SCHMIDT.  
HUBERT ALTWICKER.